# EUROPEAN PATENT SPECIFICATION

(11) **EP 3 577 270 B1**
(45) Date of publication and mention of the grant of the patent: **07.07.2021**
(21) Application number: 18707420.8
(22) Date of filing: 02.02.2018
(51) Int. Cl.: A43B 13/12, A43B 17/00, D06N 3/00, D06N 3/14, D06M 11/74

(54) **MANUFACTURED ARTICLE IN SHEET FORM, PARTICULARLY INTENDED FOR USE IN THE MANUFACTURE OF FOOTWEAR, CLOTHING ITEMS AND ACCESSORIES AND UPHOLSTERY, AND RELATED REALIZATION PROCEDURE**
HERGESTELLTER ARTIKEL IN BLATTFORM, INSBESONDERE ZUR VERWENDUNG BEI DER HERSTELLUNG VON SCHUHEN, KLEIDUNGSARTIKELN UND ACCESSOIRES UND POLSTERN, UND ZUGEHÖRIGES REALISIERUNGSVERFAHREN
ARTICLE MANUFACTURÉ SOUS FORME DE FEUILLE, DESTINÉ EN PARTICULIER À ÊTRE UTILISÉ DANS LA FABRICATION DE CHAUSSURES, D'ARTICLES ET D'ACCESSOIRES VESTIMENTAIRES ET DE REMBOURRAGES, ET PROCÉDÉ DE RÉALISATION ASSOCIÉ

(30) Priority: 03.02.2017 IT 201700012184
(43) Date of publication of application: 11.12.2019
(73) Proprietor: Fadel S.r.l., 55018 Capannori (LU) (IT)
(72) Inventor: DELLA MAGGIORA, Andrea, 55018 Capannori (LU) (IT); GIUNTOLI,Michele, 55018 Capannori (LU) (IT)
(74) Representative: Luppi, Emanuele
(86) International application number: PCT/IB2018/050663
(87) International publication number: WO 2018/142335

(56) References cited:
- EP-B1- 2 327 662
- US-A1- 2015 376 832
- DATABASE WPI Week 201660 2016 Thomson Scientific, London, GB; AN 2016-434940 XP002772583, -& CN 105 735 002 A (UNIV SICHUAN) 6 July 2016 (2016-07-06)
- DATABASE WPI Week 201577 2015 Thomson Scientific, London, GB; AN 2015-56791H XP002772584, -& CN 104 804 204 A (UNIV FUZHOU) 29 July 2015 (2015-07-29)
- DATABASE WPI Week 201629 2016 Thomson Scientific, London, GB; AN 2016-19590B XP002772585, -& CN 105 421 096 A (KUNSHAN HUAFU NEW MATERIAL CO LTD) 23 March 2016 (2016-03-23)
- DATABASE WPI Week 201656 2016 Thomson Scientific, London, GB; AN 2016-26029D XP002772586, -& CN 105 504 785 A (YINGKOU SHENGQUAN HIGH TECH MATERIAL CO) 20 April 2016 (2016-04-20)
- DATABASE WPI Week 201657 2016 Thomson Scientific, London, GB; AN 2016-26052F XP002772587, -& CN 105 504 199 A (JINAN SHENGQUAN GROUP SHARE HOLDING CO L) 20 April 2016 (2016-04-20)

## Description

### Technical Field

The present invention relates to a manufactured article in sheet form, particularly intended for use in the manufacture of footwear, clothing items and accessories, upholstery and related realization procedure.

### Background Art

The manufacture and use of cloths, fabrics, hides or other manufactured articles in sheet form are known used in the clothing, accessories and upholstery field. They are used to make footwear, leather goods, handbags, or to upholster padded parts of furniture components, car interiors and motorcyle saddles.

Such manufactured articles are made using synthetic materials, particularly polymers such as e.g. polyurethane, polyesters and PVC.

A typical example of a manufactured article in sheet form is imitation leather intended for various uses, including the production of handbags.

Imitation leather is normally made of polyurethane and can have different types of structure and finish.

Such manufactured article made of polyurethane includes among its particular features that of being lightweight, wear-resistant, water-repellent, easy to use and clean.

Traditional manufactured articles in sheet form, however, have some drawbacks.

Because they are made of polymeric materials, such manufactured articles have very little capability of dissipating heat, causing considerable discomfort to the user due to the increase in temperature perceived, especially in the hottest periods of the year.

In particular, if the manufactured article is used for the production of garments and clothing accessories, the increase in perceived temperature causes an increase in sweating, with consequent considerable discomfort.

Such drawback is particularly noticeable in the case where the manufactured article in sheet form is intended for use in the footwear sector.

In fact, the increase in temperature inside the footwear and the incorrect transpiration of the foot produce problems related to hygiene and comfort of the user.

Some types of processes for coating a sheet substrate are disclosed in the patent documents CN105735002, CN104804204 and CN105421096.

### Description of the Invention

The main aim is to provide for a manufactured article in sheet form, particularly intended for use in the manufacture of footwear, clothing items and accessories, upholstery and to its realization procedure which allow improving heat dissipation and reducing the temperature perceived by the user, which allows obtaining a high level of comfort by the user and which allows limiting perspiration due to contact with the manufacturing article and improving the hygiene, especially when used in the footwear sector and which allows also overcoming the aforementioned drawbacks of the prior art, using a simple, rational, easy, efficient to use and cost-effective solution.

The aforementioned objects are achieved by the present realization procedure of a manufactured article in sheet form, particularly intended for use in the manufacture of footwear, clothing items and accessories and upholstery, according to claim 1.

The aforementioned objects are also achieved by the present manufactured article in sheet form, particularly intended for use in the manufacture of footwear, clothing items and accessories and upholstery, according to claim 4.

### Brief Description of the Drawings

Other characteristics and advantages will become more evident from the description of a preferred embodiment of a manufactured article in sheet form, particularly intended for use in the manufacture of footwear, clothing items and accessories and upholstery, and related realization procedure, illustrated by way of an indicative example, in the attached drawings in which:
Figure 1 is an axonometric view of the step of mixing graphene with a polymeric material provided for by the procedure;
Figure 2 is an axonometric view of the step of spreading a layer of primer onto a transfer sheet provided for by the procedure;
Figure 3 is a sectional view of the step of drying for a first time the sheet provided for by the procedure;
Figure 4 is an axonometric view of the step of spreading a layer of composite material provided for by the procedure;
Figure 5 is a sectional view of the step of drying for a second time the sheet provided for by the procedure;
Figure 6 is an axonometric view of the step of spreading an adhesive layer provided for by the procedure;
Figure 7 is a sectional view of the step of drying for a third time the sheet provided for by the procedure;
Figure 8 is an axonometric view of the step of making a first main face of a substrate adhere on the adhesive layer provided for by the procedure;
Figure 9 is an axonometric view of the step of removing the transfer sheet 6 provided for by the procedure;
Figure 10 is a sectional view of the manufactured article in sheet form;
Figure 11 is an axonometric view of the manufactured article in sheet form; in a mode of use;
Figure 12 is a t/T graph of a SAMPLE 1 and related reference;
Figure 13 is a t/T graph of a SAMPLE 2 and related reference.

### Embodiments

With particular reference to Figures 1 to 9, a procedure is illustrated for the realization of a manufactured article in sheet form 1, particularly intended for use in the manufacture of footwear, clothing items and accessories and upholstery.

The procedure for the manufacture of a manufactured article in sheet form 1, particularly intended for use in the manufacture of footwear, clothing items and accessories and upholstery, comprises at least the following steps:
- a step I of mixing graphene 2 with at least a polymeric material to obtain a composite material 3; and
- a step II of applying the composite material 3 onto a substrate 4 in sheet form.

Graphene is an allotropic form of elemental carbon, consisting of a monoatomic layer of hybridized carbon atoms sp2.

It is therefore a substantially two-dimensional material, inasmuch as it has an extremely large surface area compared to its thickness, which is equal to the thickness of an atom.

Its particular structure makes it an extremely flexible material, resistant from a mechanical point of view but also with high heat conductivity.

The step I of mixing the graphene with the polymeric material permits obtaining a composite material 3, i.e. a polymeric matrix material in which the graphene 2 is dispersed.

The presence of graphene 2 in the composite material 3 changes the properties of the polymeric material, making it more resistant from a mechanical point of view, but above all conductive from a heat point of view.

Preferably, the graphene 2 is mixed with polyurethane; however, alternative solutions cannot be ruled out wherein one or more polymeric materials other than polyurethane are used.

Usefully, the step I of mixing comprises the step of adding at least one antibacterial additive selected from Echinacea extract and Tea Tree extract to the polymeric material and to the graphene, so as to improve the properties of the composite material by counteracting bacterial proliferation.

The step II of applying the composite material 3 onto the substrate 4 comprises at least the following steps:
- a step III of spreading one layer of primer 5 onto a transfer sheet 6;
- a step IV of drying the transfer sheet 6 for a first time;
- a step V of spreading the composite material 3 onto the layer of primer 5 to form at least one composite layer 7;
- a step VI of drying the transfer sheet 6 for a second time;
- a step VII of spreading an adhesive layer 8 onto the composite layer 7;
- a step VIII of drying the transfer sheet 6 for a third time;
- a step IX of making a first main face 9 of the substrate 4 adhere on the adhesive layer 8; and
- a step X of removing the transfer sheet 6.

Usefully, the transfer sheet 6 is composed of a sheet of paper having a predefined texture such as to reproduce the desired surface finish of the manufactured article in sheet form 1.

Advantageously, the step III of spreading the layer of primer 5 is done by spreading the layer of primer itself onto the transfer sheet 6 by means of a blade 11 which slides at a height set by the sheet itself.

The layer of primer 5 gives smoothness and surface resistance to the manufactured article in sheet form 1 and is made at least partly of polyurethane. After each of the steps III, V, VII of spreading, the steps IV, VI, VIII of drying the transfer sheet 6 are performed respectively in order to fix the spread material and optimize the spreading of the subsequent layer.

In particular, at least one of the step IV of drying for a first time, the step IV of drying for a second time and the step VIII of drying for a third time takes place in a kiln under the following operating conditions:
- temperature: 120 to 180 ° C
- time: 1 to 10 min.

The adhesive layer 8 used in the step VII of spreading is composed of a single-component aromatic adhesive; the use of different types of adhesive materials cannot however be ruled out.

Usefully, the adhesive layer 8 permits gluing the layers 5, 7 to the substrate 4. The step IX of making the first main face 9 of the substrate 4 adhere to the adhesive layer 8 has, therefore, the function of making the layers 5, 7 adhere and fix onto the substrate itself.

Preferably, such substrate 4 is made of coagulated polyurethane; the use of polymeric materials other than coagulated polyurethane cannot however be ruled out.

Subsequently, in step X, the transfer sheet 6 is removed, thus obtaining the manufactured article in sheet form 1.

Advantageously, the manufactured article in sheet form 1 thus obtained comprises:
- at least the substrate 4 in sheet form comprising at least the first main face 9 and at least a second main face 10; and
- at least the composite material 3 which is spread onto the first main face 9 to form the composite layer 7 and which comprises at least the polymeric material mixed with graphene.

The presence of the composite layer 7 makes the manufactured article in sheet form 1 conductive from the heat point of view.

The substrate 4 is made of breathable polyurethane, i.e. having a micro porous structure which allows for the passage of air through the substrate itself. Within the scope of this treatise, the term "breathable polyurethane" means a polyurethane having a value of permeability to water vapor above 1 mg/ (cm2 x h) measured according to the provisions of the SATRA TM 47:1997 standard. Polyurethane is one of the most versatile polymeric materials in existence and allows obtaining products with very different properties and uses.

In particular, polyurethane is a material with high resistance to mechanical stress, chemically inert with respect to very many organic and inorganic substances, resistant to humidity and to high and low temperatures.

The graphene 2 in powder form is contained in the composite material 3 in a weight percentage comprised between 0.1% and 10%.

The possibility cannot be ruled out to add the composite material 3 with at least one antibacterial additive selected from Echinacea extract and Tea Tree extract, so as to make the manufactured article in sheet form 1 antibacterial and antimicrobial.

Preferably, the manufactured article in sheet form 1 comprises at least the adhesive layer 8 interposed between the first main face 9 and the composite layer 7, so that the latter perfectly adheres to the substrate 4.

The manufactured article in sheet form 1 also comprises at least the layer of primer 5 arranged on the composite layer 7.

The manufactured article in sheet form 1 can be intended for various uses.

One possibility is to use the manufactured article in sheet form for coating at least one plate-like support 12 shaped to form an insole 13 for footwear.

The use of this insole 13 allows improving the thermal performance of the footwear, limiting the increase in the internal temperature.

Such characteristics also help limit perspiration by the user, with considerable improvement also from the hygienic point of view.

### EXAMPLE 1

A SAMPLE 1 of manufactured article in sheet form 1 was made comprising the substrate 4 in breathable polyurethane, the adhesive layer 8, the composite layer 7 and the layer of primer 5.

To make the composite layer 7 the following were used:
- graphene in the form of nanoplates (GNP), i.e. structures made up of a few sheets of carbon atoms stacked on top of each other, in a concentration by weight compared to polyurethane of 2%, in particular GNP by Strem Chemicals; and
- a non-breathable polyurethane, in particular IMAPUR 2400BV by IMA, prepared by dispersion in a solution of dimethylformamide (DMF), with the addition of isocyanates and melamine, with a concentration by weight of polyurethane between 30% and 50%.

The adhesive layer 8 was made by means of a single-component aromatic adhesive of the non-breathable type, which is ICAFLEX ADM383 by ICAP-SIRA.

To make the layer of primer 5, use was made of polyurethane IMAPUR 1500/20 HR by IMA, which is a type of non-breathable polyurethane.

The measurement was taken of the cooling speed of the SAMPLE 1 by means of an infrared camera, following radiation with a halogen lamp for a few minutes, until at least 50°C was reached.

The measurement was also taken under the same conditions on a graphene-free REFERENCE 1.

Figure 12 shows the curves describing the decrease in temperature over time, as a result of radiation, for both the SAMPLE 1 and the REFERENCE 1.

The cooling speed is determined by the initial slope of the cooling curve.

It was noted that the cooling speed was the same for the two samples examined.

The maximum temperature (T_{MAX}) recorded is shown on Table 1.

**Table 1**

| | T_{MAX} |
|---|---|
| SAMPLE 1 | 62.1°C |
| REFERENCE 1 | 60.7°C |

It was noted that the T_{MAX} reached by SAMPLE 1 was higher than the T_{MAX} reached by REFERENCE 1.

The higher T_{MAX} is linked to the presence of graphene in the composite material 3, which improves its heat conductivity; however, the use of non-breathable materials means that there are no changes as regards heat dissipation.

### EXAMPLE 2

A SAMPLE 2 of manufactured article in sheet form 1 was made comprising the substrate 4 in breathable polyurethane, the adhesive layer 8, the composite layer 7 and the layer of primer 5.

In this case, to make the composite layer 7 the following were used:
- graphene in the form of nanoplates (GNP), in a concentration by weight compared to polyurethane of 2%, in particular GNP by Strem Chemicals; and
- a breathable polyurethane, in particular NORETHANE NPU511 by NOVOTEX, prepared by dispersion in a solution of dimethylformamide (DMF), with the addition of isocyanates and melamine, with a concentration by weight of polyurethane between 30% and 50%.

The adhesive layer 8 was made by means of a single-component breathable adhesive, which is LARITHANE AB7198 by NOVOTEX.

To make the layer of primer 5 a material was used identical to that used to make the composite layer 7, i.e., polyurethane NORETHANE NPU511 by NOVOTEX to which graphene GNP by Strem Chemicals was mixed in a concentration by weight of 2%.

In this case too, a measurement test was performed of the cooling speed of the SAMPLE 2, carried out according to the same specifications shown for the SAMPLE 1, comparing the results with a REFERENCE 2 comprising the same materials, but free of graphene.

Figure 13 shows the curves that describe the temperature trend over time as a consequence of irradiation, both for the SAMPLE 2 and for the REFERENCE 2.

In this case the cooling speed of the SAMPLE 2 is slightly higher with respect to the REFERENCE 2.

The maximum temperature (T_{MAX}) recorded is shown on Table 2.

**Table 2**

| | T_{MAX} |
|---|---|
| SAMPLE 2 | 57.0°C |
| REFERENCE 2 | 61.2°C |

In this second case, the T_{MAX} reached by SAMPLE 2 was lower than the T_{MAX} reached by REFERENCE 2.

This result is due to the fact that the graphene contained in both the layer of primer 5 and in the composite layer 7 makes it possible to obtain a more uniform distribution of the Ts, with lower maximum temperature.

Furthermore, the use of breathable materials makes it possible to dissipate heat more quickly than in the previous case, increasing the action performed by the graphene.

It has in practice been found hereby how to achieve the intended objects.

In this regard, it is underlined that the special solution of providing a composite layer containing graphene makes it possible to improve heat dissipation. Furthermore, the special solution of mixing graphene with breathable polyurethane allows reducing the temperature perceived by the user and obtaining a high level of comfort for the user, especially during hot periods. Still furthermore, the use of the manufactured article in sheet form for covering shoe insoles makes it possible to reduce perspiration by the user, with a considerable improvement also from the hygienic point of view.

## Claims

1. Procedure for the manufacture of a manufactured article in sheet form (1), particularly intended for use in the manufacture of footwear, clothing items and and accessories and upholstery, comprising at least the following steps:
- mixing (I) graphene (2) with at least a polymeric material to obtain a composite material (3); and
- applying (II) said composite material (3) onto a substrate (4) in sheet form; **characterized by** the fact that said applying comprises at least the steps of:
- spreading (III) a layer of primer (5) onto a transfer sheet (6);
- drying (IV) said transfer sheet (6) for a first time;
- spreading (V) said composite material (3) onto said layer of primer (5) to form at least a composite layer (7);
- drying (VI) said transfer sheet (6) for a second time;
- spreading (VII) an adhesive layer (8) on said composite layer (7);
- drying (VIII) said transfer sheet (6) for a third time;
- making a first main face (9) of said substrate (4) adhere (IX) on said adhesive layer (8); and
- removing (X) said transfer sheet (6).

2. Procedure according to claim 1, **characterized by** the fact that said mixing (I) comprises the step of adding at least an antibacterial additive selected from Echinacea extract and Tea Tree extract to said polymeric material and to said graphene (2).

3. Procedure according to one or more of the preceding claims, **characterized by** the fact that at least one of said drying for a first time (IV), said drying for a second time (VI) and said drying for a third time (VIII) takes place under the following operating conditions:
- temperature: 120 to 180 ° C
- time: 1 to 10 min.

4. Manufactured article in sheet form (1), particularly intended for use in the manufacture of footwear, clothing items, accessories and upholstery, manufactured by means of the procedure according to one or more of claims 1 to 3, wherein it comprises:
- at least a substrate (4) in sheet form comprising at least a first main face (9) and at least a second main face (10); and
- at least a composite material (3) spread onto said first main face (9) to form a composite layer (7) and comprising at least a polymeric material mixed with graphene (2).

5. Manufactured article in sheet form (1) according to claim 4, **characterized by** the fact that said substrate (4) is made of breathable polyurethane.

6. Manufactured article in sheet form (1) according to claim 4 or 5, **characterized by** the fact that said polymeric material is polyurethane.

7. Manufactured article in sheet form (1) according to one or more of claims 4 to 6, **characterized by** the fact that said graphene (2) is contained in said composite material (3) in a weight percentage comprised between 0.1% and 10%.

8. Manufactured article in sheet form (1) according to one or more of claims 4 to 7, **characterized by** the fact that said composite material (3) comprises at least an antibacterial additive selected from Echinacea extract and Tea Tree extract.

9. Manufactured article in sheet form (1) according to one or more of claims 4 to 8, **characterized by** the fact that it comprises:
- at least an adhesive layer (8) interposed between said first main face (9) and said composite layer (7); and
- at least a layer of primer (5) arranged on said composite layer (7).

10. Use of the manufactured article in sheet form (1) according to one or more of claims 4 to 9, for coating at least a plate-like support (12) shaped to form an insole (13) for footwear.

## Patentansprüche

1. Verfahren zur Herstellung eines blattförmigen Erzeugnisses (1), das insbesondere zur Verwendung bei der Herstellung von Schuhen, Kleidungsstücken und Zubehör sowie Polstermöbeln bestimmt ist, umfassend mindestens die folgenden Schritte:
- Mischen von (I) Graphen (2) mit mindestens einem polymeren Material, um ein Verbundmaterial (3) zu erhalten; und
- Auftragen (II) des Verbundmaterials (3) auf ein Substrat (4) in Blattform;
**dadurch gekennzeichnet, dass**
das Auftragen mindestens die folgenden Schritte umfasst:
- Aufbringen (III) einer Schicht Grundierung (5) auf eine Transferfolie (6);
- Trocknen (IV) der Transferfolie (6) zum ersten Mal;
- Aufbringen (V) des Verbundmaterials (3) auf die Schicht der Grundierung (5), um mindestens eine Verbundschicht (7) zu bilden;
- Trocknen (VI) der Transferfolie (6) zum zweiten Mal;
- Aufbringen (VII) einer Klebstoffschicht (8) auf die Verbundschicht (7);
- Trocknen (VIII) der Transferfolie (6) zum dritten Mal;
- Veranlassen, dass eine erste Hauptfläche (9) des Substrats (4) an der Klebstoffschicht (8) haftet (IX); und
- Entfernen (X) der Transferfolie (6).

2. Verfahren nach Anspruch 1, **dadurch gekennzeichnet, dass** das Mischen (I) den Schritt der Zugabe mindestens eines antibakteriellen Zusatzes aus Echinacea-Extrakt und Teebaum-Extrakt zu dem polymeren Material und zu dem Graphen (2) umfasst.

3. Verfahren nach einem oder mehreren der vorhergehenden Ansprüche, **dadurch gekennzeichnet, dass** mindestens einer der Vorgänge des Trocknens zum ersten Mal (IV), des Trocknens zum zweiten Mal (VI) und des Trocknens zum dritten Mal (VIII) unter den folgenden Betriebsbedingungen stattfindet:
- Temperatur : 120 bis 180°C
- Zeit : 1 bis 10 min.

4. Blattförmiges Erzeugnis (1), insbesondere zur Verwendung bei der Herstellung von Schuhen, Kleidungsstücken, Zubehör und Polstermöbeln, hergestellt mittels des Verfahrens nach einem der Ansprüche 1 bis 3, wobei dieses umfasst:
- mindestens ein blattförmiges Substrat (4) mit mindestens einer ersten Hauptfläche (9) und mindestens einer zweiten Hauptfläche (10); und
- mindestens ein Verbundmaterial (3), das auf die erste Hauptfläche (9) aufgetragen wird, eine Verbundschicht (7) bildet und mindestens ein mit Graphen (2) gemischtes polymeres Material umfasst.

5. Blattförmiges Erzeugnis (1) nach Anspruch 4, **dadurch gekennzeichnet, dass** das Substrat (4) aus atmungsaktivem Polyurethan hergestellt ist.

6. Blattförmiges Erzeugnis (1) nach Anspruch 4 oder 5, **dadurch gekennzeichnet, dass** das polymere Material Polyurethan ist.

7. Blattförmiges Erzeugnis (1) nach einem der Ansprüche 4 bis 6, **dadurch gekennzeichnet, dass** das Graphen (2) in dem Verbundmaterial (3) in einem Gewichtsprozentanteil zwischen 0,1% und 10 % enthalten ist.

8. Blattförmiges Erzeugnis (1) nach einem der Ansprüche 4 bis 7, **dadurch gekennzeichnet, dass** das Verbundmaterial (3) mindestens einen antibakteriellen Zusatz aus Echinacea-Extrakt und Teebaumextrakt enthält.

9. Blattförmiges Erzeugnis (1) nach einem der Ansprüche 4 bis 8, **gekennzeichnet durch**
- mindestens eine Klebeschicht (8), die zwischen der ersten Hauptfläche (9) und der Verbundschicht (7) angeordnet ist; und
- mindestens eine auf der Verbundschicht (7) angeordnete Schicht aus Grundierung (5).

10. Verwendung des blattförmigen Erzeugnisses (1) nach einem der Ansprüche 4 bis 9 zum Beschichten mindestens eines plattenförmigen Trägers (12), der so geformt ist, dass er eine Einlegesohle (13) für Schuhe bildet.

## Revendications

1. Procédure pour la fabrication d'un article manufacturé sous forme de feuille (1), en particulier destiné à être utilisé dans la fabrication de chaussures, d'articles et d'accessoires et de rembourrages vestimentaires, comprenant au moins les étapes suivantes :
- mélange (I) de graphène (2) avec au moins un matériau polymère pour obtenir un matériau composite (3) ; et
- application (II) dudit matériau composite (3) sur un substrat (4) sous forme de feuille ;
**caractérisée par le fait que** ladite application comprend au moins les étapes de :
- étalement (III) d'une couche d'apprêt (5) sur une feuille de transfert (6) ;
- séchage (IV) de ladite feuille de transfert (6) pendant un premier temps ;
- étalement (V) dudit matériau composite (3) sur ladite couche d'apprêt (5) pour former au moins une couche composite (7) ;
- séchage (VI) de ladite feuille de transfert (6) pendant un deuxième temps ;
- étalement (VII) d'une couche adhésive (8) sur ladite couche composite (7) ;
- séchage (VIII) de ladite feuille de transfert (6) pendant un troisième temps ;
- adhérence (IX) d'une première face principale (9) dudit substrat (4) sur ladite couche adhésive (8) ; et
- retrait (X) de ladite feuille de transfert (6).

2. Procédure selon la revendication 1, **caractérisée par le fait que** ledit mélange (I) comprend l'étape d'ajout d'au moins un additif antibactérien sélectionné parmi un extrait d'échinacée et un extrait d'arbre à thé audit matériau polymère et audit graphène (2).

3. Procédure selon une ou plusieurs des revendications précédentes, **caractérisée par le fait qu'**au moins un parmi ledit séchage pendant un premier temps (IV), ledit séchage pendant un deuxième temps (VI) et ledit séchage pendant un troisième temps (VIII) a lieu dans les conditions de fonctionnement suivantes :
- température : de 120 à 180 °C
- temps : 1 à 10 min.

4. Article manufacturé sous forme de feuille (1), en particulier destiné à être utilisé dans la fabrication de chaussures, d'articles, d'accessoires et de rembourrages vestimentaires, fabriqué à l'aide de la procédure selon une ou plusieurs des revendications 1 à 3, ledit article manufacturé comprenant :
- au moins un substrat (4) sous forme de feuille comprenant au moins une première face principale (9) et au moins une seconde face principale (10) ; et
- au moins un matériau composite (3) étalé sur ladite première face principale (9) pour former une couche composite (7) et comprenant au moins un matériau polymère mélangé à du graphène (2).

5. Article manufacturé sous forme de feuille (1) selon la revendication 4, **caractérisé par le fait que** ledit substrat (4) est composé de polyuréthane respirable.

6. Article manufacturé sous forme de feuille (1) selon la revendication 4 ou 5, **caractérisé par le fait que** ledit matériau polymère est du polyuréthane.

7. Article manufacturé sous forme de feuille (1) selon une ou plusieurs des revendications 4 à 6, **caractérisé par le fait que** ledit graphène (2) est contenu dans ledit matériau composite (3) en un pourcentage en poids compris entre 0,1 % et 10 %.

8. Article manufacturé sous forme de feuille (1) selon une ou plusieurs des revendications 4 à 7, **caractérisé par le fait que** ledit matériau composite (3) comprend au moins un additif antibactérien sélectionné parmi un extrait d'échinacée et un extrait d'arbre à thé.

9. Article manufacturé sous forme de feuille (1) selon une ou plusieurs des revendications 4 à 8, **caractérisé par le fait qu'**il comprend :
- au moins une couche adhésive (8) intercalée entre ladite première face principale (9) et ladite couche composite (7) ; et
- au moins une couche d'apprêt (5) agencée sur ladite couche composite (7).

10. Utilisation de l'article manufacturé sous forme de feuille (1) selon une ou plusieurs des revendications 4 à 9, pour recouvrir au moins un support en forme de plaque (12) façonné pour former une semelle intérieure (13) pour chaussure.
